

## UNITED STATES PATENT OFFICE.

EDWARD C. HOLTON, OF CLEVELAND, OHIO, ASSIGNOR OF ONE-HALF TO THE SHERWIN-WILLIAMS COMPANY, OF CLEVELAND, OHIO, A CORPORATION OF OHIO.

## PROCESS OF PRODUCING PAINT-OIL.

SPECIFICATION forming part of Letters Patent No. 728,918, dated May 26, 1903.

Application filed September 25, 1902. Serial No. 124,826. (No specimens.)

*To all whom it may concern:*

Be it known that I, EDWARD C. HOLTON, a citizen of the United States, and a resident of Cleveland, county of Cuyahoga, and State of Ohio, have invented a new and useful Improvement in Processes of Producing Paint-Oils, of which the following is a specification, the principle of the invention being herein explained and the best mode in which I have contemplated applying that principle, so as to distinguish it from other inventions.

My invention relates to processes of producing paint-oils, and more particularly to that class of oils which are used as substitutes for linseed-oil, and has for its object the production of such substitutes in a manner more efficacious and economical than that of the methods hitherto employed.

Heretofore oils with the drying qualities of linseed-oil and intended as a substitute for that oil have been prepared from a limited number of animal and vegetable oils diluted with varying amounts of some petroleum product or some other solvent by treating same with from fifteen to thirty per cent. of sulfur chlorid, the amount depending upon the nature of the oil. The difficulty connected with this method has been that most animal and vegetable oils when thus treated with sulfur chlorid are rendered solid and are not then soluble in those solvents which are usually employed for thinning paint products. Furthermore, those few oils which are soluble in the usual solvents which are employed for paint products require so much sulfur chlorid before the proper drying qualities are imparted to them that the cost of the finished product is materially greater than that sustained in the production of such substitutes in the manner that I shall hereinafter describe.

In my improved process I do not use the raw oils, but those oils that have been blown, the production of which is a process familiar to any one skilled in the art and the claim for the invention in the method of doing which forms no part of this application. With these blown oils I mix by simply agitating from one-half to one per cent. of sulfur chlorid in solution in a hydrocarbon. It is very essen-

tial that the sulfur chlorid be diluted with a hydrocarbon before being mixed with the blown oil, to what extent, however, will be hereinafter described, since otherwise the action would be too violent and would effect a 55 localized and imperfect result. To the mixture of blown oil and solution of sulfur chlorid in hydrocarbon I add approximately an equal amount of kerosene or some other petroleum product, thinning the resultant oil, if it be 60 still too thick, with some cheap solvent belonging to the hydrocarbons of the paraffin series, preferably benzin, or I may use a hydrocarbon belonging to the benzole series. These solvents may be added either before or after 65 the treatment with the solution of sulfur chlorid and hydrocarbon. The amount of hydrocarbon used with the sulfur chlorid previous to mixing with the blown oil will depend upon atmospheric and other conditions readily understood by those skilled in the art. In cold weather it would be preferable to use a greater amount of hydrocarbon with the sulfur chlorid before mixing with the blown oil than in warm weather. Again, if the 70 agitation of the sulfur chlorid with the blown oil was to be made with a powerful mechanical agitator a smaller amount of hydrocarbon would be required than if a less powerful agitator were used. It may occur under cer- 75 tain conditions that it would be the best practice to mix the sulfur chlorid with the whole amount of kerosene before mixing with the blown oil. Experiment has proved that a mixture of approximately twenty parts of 80 hydrocarbon to one of sulfur chlorid is the most effective under normal atmospheric conditions; but the existing conditions at the time of mixing must be observed in order to 85 secure the best results, and the details must 90 be left to the good judgment and skill of the operator, the broad idea merely involving the treatment of blown oils with sulfur chlorid in solution with a hydrocarbon. By thus using 95 blown oils instead of the raw products all vegetable and animal oils can be utilized, because the amount of sulfur chlorid that is then necessary to produce the drying qualities required in the finished product is com- 100 paratively so small that the oil is turned into

a mass which is soft and pliable, like rubber, and not into the solid body which is produced by the use of fifteen per cent. or more of sulfur chlorid and which solid body is soluble 5 in the ordinary solvents used for thinning paints in the case of only a very few oils, as has been heretofore mentioned.

The material reduction in the cost of production of the finished product by the use of 10 one per cent. of sulfur chlorid instead of fifteen per cent. or more is very evident.

I am aware that some oils other than linseed-oil are blown and that there are commercial products upon the market under the 15 term "blown oil;" but they are used for special purposes in special cases only and are not offered for sale for any particular use, and, furthermore, in no case are they utilized in the manner heretofore described and here- 20 inafter claimed in my application.

Other modes of applying the principle of my invention may be employed instead of the one explained, change being made as regards the process herein disclosed, provided 25 the means stated by any one of the following claims or the equivalent of such stated means be employed.

I therefore particularly point out and distinctly claim as my invention—

1. A step in a method of producing paint- 30 oils, consisting of: treating blown oils with sulfur chlorid in solution in a hydrocarbon.

2. Steps in a method of producing paint- 35 oils, consisting of: treating blown oils with sulfur chlorid in solution in a hydrocarbon, and thinning this mixture with some petro- leum product.

3. Steps in a method of producing paint- 40 oils, consisting of: treating blown oils with approximately one per cent. of sulfur chlorid in solution in approximately twenty parts of a hydrocarbon, diluting this product with an amount of some petroleum product approximately equal to the mixture of blown oil and solution of sulfur chlorid in hydrocarbon, and 45 thinning the resultant mixture with benzine down to a consistency where it can be used for the purpose specified.

Signed by me this 23d day of September, 1902.

EDWARD C. HOLTON.

Attest:

D. T. DAVIES,  
GEO. W. SAYWELL.